

Oct. 12, 1926.

1,602,595

S. E. SHEPPARD ET AL

ELECTROLYTICAL PROCESS OF PREPARING SILVER HALIDES FROM METALLIC SILVER

Filed Feb. 27, 1926

FIG. 1.



FIG. 2.



FIG. 3.



## UNITED STATES PATENT OFFICE.

SAMUEL E. SHEPPARD AND RAYMOND H. LAMBERT, OF ROCHESTER, NEW YORK, ASSIGNEES TO EASTMAN KODAK COMPANY, OF ROCHESTER, NEW YORK, A CORPORATION OF NEW YORK.

ELECTROLYTICAL PROCESS OF PREPARING SILVER HALIDES FROM METALLIC SILVER.

Application filed February 27, 1926. Serial No. 91,815.

This invention relates to electrolytic processes of preparing silver halides from metallic silver. One object of the invention is to provide a simplified process which will avoid expensive operations now used in preparing such halides. Another object is to provide a process in which the formation of intermediate silver compounds is unnecessary. A still further object is to provide a process for preparing such halides in a fine-grained, deflocculated form readily purified by washing and suitable for photographic or pharmaceutical purposes. Another object of the invention is to provide an electrolytic process for preparing halides in which the electrolyte passes through a cycle which avoids waste of silver values. Yet another object of the invention is to provide an electrolytic process in which alkalization of the anolyte is usefully opposed. Other objects will hereinafter appear.

In the accompanying drawing.—

Fig. 1 is a diagrammatic vertical sectional view, upon an exaggerated scale, of an apparatus in which our process may be carried out;

Fig. 2 is a diagrammatic vertical sectional view of another form of apparatus in which our process may be carried out;

Fig. 3 is a mill diagram illustrating one form of our process.

Silver halides for photographic and pharmaceutical use are usually prepared by precipitation when a solution of a soluble silver salt has been mixed with a solution of a soluble halide. The soluble silver salt which is most commonly employed is the nitrate. The preparation of this salt in a pure form requires that the silver be dissolved in nitric acid of stringent chemical purity. From this solution silver nitrate is obtained by tedious crystallization and recrystallization. Our process avoids this production of an intermediate salt together with its tedious and expensive operations.

After the pure silver nitrate is dissolved and silver halides are precipitated, from this solution, such halides must be very thoroughly washed. We have found that the silver halides produced by our process may be washed free from the associated products of the reaction more easily than in the case of the silver halides produced in the conventional manner.

Our process is concerned with silver bromide, silver iodide and silver chloride and not with silver fluoride. Since bromide, iodine and chlorine are all of higher atomic weight than fluorine, we shall, for convenience, hereinafter designate them as a group, as well as their silver and other compounds, by the adjective "heavy",—thus a "heavy" halide of silver means either silver bromide, iodide, or chloride and not the fluoride.

We have discovered that the hereinabove recited objects may be attained in the preparation of the heavy halides of silver by converting anode silver into such halides in aqueous electrolytes which are solvents of such heavy silver halides and contain heavy halide anions. The heavy halide which is formed from the anode silver by electrolysis dissolves in the electrolyte. When the latter has taken up a practical proportion of the heavy silver halide, it is treated so that its solvent power is reduced, in order to precipitate fine-grained and deflocculated silver halide. This is readily separated from the electrolyte and thoroughly washed with water. In the preferred form of our invention the solvent power and the anion content of the electrolyte are then restored to normal so that it can be reused in treating further anode silver. In this way the process may be made continuous by passing the electrolyte through this circle, and waste of heavy halide anions is practically eliminated, as well as waste of unprecipitated silver halide.

The electrolytes which we prefer are solvents of the heavy silver halides by reason of their concentrated content of one or more of the heavy halides of the alkali metals, or by reason of the high temperature of the electrolyte, or preferably both. We shall hereinafter include in the term "alkali metal" ammonium the salts of which function, in our process, in the same way that the salts of the alkali metals do. The heavy halide alkali salt or salts which are present in the electrolyte, correspond to the heavy silver halide or halides to be produced. Thus when making silver bromide we employ a hot concentrated bath of a bromide of an alkali metal. It is preferable to use saturated solutions of the alkali salts and to maintain them during the electrolysis at a

temperature between 70° C. and boiling. We have found 80° C. to be convenient, but temperatures up to the boiling point of the solution may be used to give heavier yields.

While the principle of the process is applicable to the production of silver chloride, as well as silver bromide and silver iodide, the process is much more easily carried out in the case of the two latter compounds, because it is easier to prepare suitable electrolytes for their production which have the necessary solvent power.

Since silver bromide is of the widest technical importance, we shall give examples of our process in the manufacture of this compound, but it will be understood that our invention is not restricted to the details thus given, except as indicated in the appended claims.

Referring to Figure 1, in the vessel 1 is located the electrolyte 2. This may be, for example, a saturated aqueous solution of potassium bromide heated to 80° C. in any suitable manner, say by burner 3. Suspended in the electrolyte are the metallic silver anode 4 and cathode 5. The cathode may be of any conductor which will not contaminate the bath, but a silver cathode gives good results and high current efficiency. The current may be direct or even a pulsating current obtained by superposing an alternating current upon a direct current. The current density may be varied over a considerable range. It is not essential that it be kept uniform throughout the electrolysis, so long as it is maintained within practical limits. An initial current density of 6.5 amperes per square decimeter illustrates a good average value. In the arrangement shown in Figure 1, this current density tends to rise during the electrolysis, where constant current is maintained by suitable regulators, because the area of the anode is progressively decreased as it dissolves away. As is well known in the art, a constant current density can be maintained by feeding bar anodes into the electrolyte either by hand or automatically. As such devices are well known, no description of them is needed.

The electrolysis is carried on until the electrolyte is practically saturated with silver bromide, which is dissolved by the bath as fast as it is formed at the anode. The end point can be indicated by testing the electrolyte at intervals, or by noting the appearance of the anode when the silver bromide is not dissolved with sufficient rapidity. When the content of silver bromide in the electrolyte has reached a practical amount the electrolyte is drawn out, say through valve 6, and both cooled and diluted with water, preferably at or below room temperature.

This causes a fine-grained flocculent precipitate of bromide which may be readily separated from the electrolyte, by settling and decantation, or by filtering, or by any other of the known processes of separating liquids and their precipitates. Filtering is convenient and the filtered silver bromide is easily washed substantially free from potassium bromide and any other salts present or formed in the electrolyte during the process. We have found that a precipitate, obtained in the manner indicated above, is purified especially readily with the minimum amount of washing. Plain cold water is effective, although after the bulk of the potassium bromide is washed away, warm water may be employed in the purification, if desired. Minimum washing lessens loss of silver values.

The diluted electrolyte is then restored to substantially its initial condition by re-heating it to 80° C. and resaturating it with potassium bromide. This makes it ready for the further treatment of anode silver. The bath thus functions through a regular cycle. This brings about a very important saving, because any silver bromide which is not precipitated out from it is restored to the electrolysis vessel, and thus there is no leak of silver values. Potassium bromide may be added, or water driven off, or both, when resaturating the bath.

During each electrolytic operation the catholyte around the cathode 5 becomes basic in character. The hydroxyl ions thus produced, may, in time, migrate into the anolyte and interfere with the production of silver bromide and its dissolution in the bath. We have found that this can be corrected by stirring in small amounts of hydrobromic acid, as needed, to keep the anolyte in proper condition free from excessive alkalinity. We have indicated a source of hydrobromic acid diagrammatically at 7 in Figure 1. In this way practically 100% current efficiency can be maintained.

We can not only oppose the alkalinization of the anolyte by neutralizing with the proper heavy halide acid, but can likewise oppose it by using a suitable porous diaphragm. The layout of such a system is shown diagrammatically in Figure 2. In this view the vessel 8 contains the electrolyte 9, which may be a saturated solution of potassium bromide, as in the apparatus of Figure 1. The anolyte and catholyte may be initially the same. The electrolyte may be maintained at suitable temperature, say 80° C. by heating jacket 10, in which steam, hot water, heated oil or other heat carrier may be employed. The porous diaphragm is indicated at 11 conventionally supported at 12. It may be cylindrical with the silver anodes 13 arranged around it. While any kind of porous diaphragm, not

attacked by hot solutions of the salts used, are suitable, we prefer unglazed porcelain, alundum, sintered glass or the like. Any suitable cathode 14 may be employed. When 5 the content of silver bromide has increased to a desirable proportion in the electrolyte, the latter may be drawn off through valve 15. In case an undue portion of hydroxyl ions migrate through the diaphragm 11 into 10 the anolyte surrounding anodes 13, said anolyte may be acidified by using hydrobromic acid, a source of this material being diagrammatically indicated at 16. It will be evident that the adding of regenerated electrolyte to the vessel 1, and the withdrawal 15 of the silver-bromide-loaded electrolyte therefrom may take place simultaneously so as to make a continuous process. Moreover, the anodes may be fed into the bath automatically in any suitable way. We prefer 20 to move or agitate the electrolyte adjacent the anode where the silver halide is formed and dissolved. In the drawing we have conventionally represented electric motors 25 17 geared to stirrers 18.

When preparing silver bromide by our process, we have found that over 6% of the silver bromide may be dissolved in the saturated silver bromide at 80° C. and over 10% 30 at 100° C., which is sufficient to be technically important and usable. This may be slightly below saturation at the temperature employed but is, nevertheless, practical. When the electrolyte is both cooled and diluted the loss in solvent power toward silver bromide is very marked and a good extraction by precipitation is, therefore, possible. For dilution we use water free from troublesome impurities, say distilled water.

40 The process, especially when preparing heavy halides of silver for photographic use, is preferably carried out in non-actinic or "safe" light, of a suitable yellow or red color. The electrolysis may be carried out in ordinary daylight or the usual artificial lights, the precipitation and all subsequent steps should be done in a safely lighted room.

Having thus described our invention, what 50 we claim as new and desire to secure by Letters Patent is:

1. The process of preparing a heavy halide of silver which includes the steps of electrolytically converting anode silver into silver halide in an aqueous electrolyte which 55 is a solvent of said silver halide and contains heavy halide anions, reducing the solvent power of said electrolyte to precipitate silver halide dissolved during said first-named step, and separating the precipitate from 60 said electrolyte.

2. The cyclic process of preparing a heavy halide of silver which includes the steps of electrolytically converting anode silver into silver halide in an aqueous electrolyte which 65 is a solvent of said silver halide and contains

heavy halide anions, reducing the solvent power of said electrolyte to precipitate silver halide dissolved during said first-named step, separating the precipitate from said electrolyte, and restoring the solvent power and 70 halide anion content of said electrolyte for treating further anode silver.

3. The process of preparing a heavy halide of silver which includes the steps of electrolytically converting anode silver into silver 75 halide in an aqueous electrolyte containing heavy halide anions heated above room temperature, said electrolyte having greater solvent power above room temperature than at or below room temperature for said silver halide, lowering the temperature of said electrolyte until silver halide dissolved during said first step is precipitated, separating the precipitate from said electrolyte, and purifying it by washing.

4. The process of preparing a heavy halide of silver which includes the steps of electrolytically converting anode silver into silver halide in an aqueous electrolyte containing heavy halide anions heated above room temperature, said electrolyte having greater solvent power above room temperature than at or below room temperature for said silver halide, lowering the temperature of said electrolyte until silver halide dissolved during said first step is precipitated, separating the precipitate from said electrolyte, and purifying it by washing, the halide anion content and the temperature of said electrolyte being thereafter restored for the treatment of further anode silver.

5. The process of preparing a heavy halide of silver which includes the step of electrolytically converting anode silver into silver halide in an aqueous electrolyte substantially saturated with the corresponding heavy halide of an alkali metal above room temperature, cooling and diluting said electrolyte to precipitate silver halide dissolved during said first-named step, and separating the precipitate from said electrolyte.

6. The process of preparing a heavy halide of silver which includes the steps of electrolytically converting anode silver into silver halide in an aqueous electrolyte containing heavy halide anions heated above room temperature, said electrolyte having greater solvent power above room temperature than at or below room temperature for said silver halide, lowering the temperature of said electrolyte until silver halide dissolved during said first step is precipitated, separating the precipitate from said electrolyte, and purifying it by washing, the halide anion content and the temperature of said electrolyte being thereafter restored for the treatment of further anode silver, said electrolyte being thereafter resaturated with said alkali halide and restored in temperature for the treatment of further anode silver.

7. The process of preparing silver bromide which includes the steps of electrolytically converting anode silver into silver bromide in an aqueous electrolyte which is a solvent of silver bromide and contains bromide ions, reducing the solvent power of said electrolyte to precipitate silver bromide dissolved during said first-named step, and separating the precipitate from said electrolyte.

8. The process of preparing silver bromide which includes the steps of electrolytically converting anode silver into silver bromide in an aqueous electrolyte which is a solvent of silver bromide and contains bromide ions, reducing the solvent power of said electrolyte to precipitate silver bromide dissolved during said first-named step, and separating the precipitate from said electrolyte, the solvent power and bromide ion content of said electrolyte being restored for treatment of further anode silver.

9. The process of preparing silver bromide which comprises the step of electrolytically attacking a silver anode in an aqueous electrolyte having sufficiently high bromide ion concentration to dissolve the resulting silver bromide as it is formed.

10. The process of preparing silver bromide which comprises the step of electrolytically attacking anode silver in an aqueous electrolyte of alkali bromide heated above room temperature which dissolves the resulting silver bromide as it is formed.

11. The process of preparing a heavy halide of silver which includes the step of electrolytically dissolving a silver anode in an electrolyte comprising a saturated aqueous solution of a heavy halide of an alkali metal at a temperature from 70° C. to boiling.

12. The process of preparing silver bromide which includes electrolytically dissolving a silver anode in an electrolyte comprising an aqueous saturated solution of an alkali bromide at a temperature from 70° C. to boiling, and precipitating, separating and washing the resulting silver bromide from said solution.

13. The cyclic process of preparing silver bromide which includes electrolytically dissolving a silver anode in an electrolyte comprising initially an aqueous saturated solution of an alkali bromide at a temperature from 70° C. to boiling, precipitating and separating the resulting silver bromide from said solution, and bringing said electrolyte to its initial condition for treating further silver anodes.

14. The process of preparing a heavy halide of silver which includes the steps of electrolytically converting anode silver into said silver halide in an aqueous electrolyte containing sufficient corresponding heavy halide of an alkali metal to dissolve said

silver halide, and opposing alkalization of the anolyte by the catholyte.

15. The process of preparing a heavy halide of silver which includes the steps of electrolytically converting anode silver into said silver halide in an aqueous electrolyte containing sufficient corresponding heavy halide of an alkali metal to dissolve said silver halide, and adding the corresponding heavy halide acid to the electrolyte.

16. The process of preparing a heavy halide of silver which includes the steps of electrolytically converting anode silver into said silver halide in an anolyte containing sufficient corresponding heavy halide of an alkali metal to dissolve said silver halide, said anolyte being separated by a porous diaphragm from the catholyte.

17. The process of preparing silver bromide which includes the steps of electrolytically attacking anode silver in an aqueous electrolyte containing sufficient alkali bromide to dissolve the silver bromide, and opposing alkalization of the anolyte by the catholyte.

18. The process of preparing silver bromide which includes the steps of electrolytically attacking anode silver in an anolyte of aqueous alkali bromide solution said anolyte being sufficiently concentrated and heated to dissolve the silver bromide thus formed, and adding hydrobromic acid to said anolyte.

19. The process of preparing silver bromide which includes the steps of electrolytically attacking anode silver in an electrolyte of aqueous alkali bromide solution, the anolyte being separated from the catholyte by a porous diaphragm and said anolyte being sufficiently concentrated and heated to dissolve the silver bromide thus formed.

20. The process of preparing silver bromide which includes the steps of electrolytically attacking anode silver in an electrolyte of saturated aqueous alkali bromide solution, the anolyte being separated from the catholyte by a porous diaphragm and said anolyte being heated between 70° C. and boiling.

21. The process of preparing silver bromide which includes the steps of electrolytically attacking anode silver in an electrolyte of saturated aqueous alkali bromide solution, the anolyte being separated from the catholyte by a porous diaphragm and said anolyte being heated between 70° C. and boiling, and adding hydrobromic acid to said anolyte to counteract alkali migration through the diaphragm from the catholyte.

Signed at Rochester, New York, this 22nd day of February, 1926.

SAMUEL E. SHEPPARD.  
RAYMOND H. LAMBERT.